



DANIEL M. CUMMINGS, OF ENFIELD, NEW HAMPSHIRE, ASSIGNOR TO HIMSELF AND  
WASHINGTON IRVING CONANT, OF SAME PLACE.

*Letters Patent No. 85,216, dated December 22, 1868.*

IMPROVED COMPOSITION FOR WATER-PROOF PAINT, &c.

The Schedule referred to in these Letters Patent and making part of the same.

*To all whom it may concern:*

Be it known that I, DANIEL M. CUMMINGS, of Enfield, in the county of Grafton, and State of New Hampshire, have invented a new and improved Composition of Matter in the Shape of a Water-Proof Painting or Coating-Mixture; and I do hereby declare the following to be a full and exact description of the method of producing the same.

The said mixture is composed of clay, tar, oil, ashes, and oxide of iron, in about the following proportions, viz:  $\frac{60}{100}$  clay;  $\frac{30}{100}$  tar;  $\frac{2}{100}$  oil;  $\frac{4}{100}$  ashes, and  $\frac{4}{100}$  oxide of iron.

These ingredients, when thoroughly incorporated with each other, will produce a perfectly water-proof coating for street-sidewalks, roofs, cisterns, basement-floors, sewers, &c.; and when reduced to the proper

consistence, by the addition of oil or other suitable fluid, it can be employed as a water-proof paint, for the painting of any exposed surfaces of wood, metal, cloth, &c.

What I claim as my invention, and desire to secure by Letters Patent, as a new composition of matter, is—

A water-proof coating or painting-mixture, composed of clay, tar, oil, ashes, and oxide of iron, in about the proportions herein described.

The foregoing specification of my improved composition of matter, for painting and other purposes, signed and witnessed, this 16th day of November, 1868.

DANIEL M. CUMMINGS.

Witnesses:

WILLIAM MORSE,  
JAMES F. PATTEE.